

2,936,229

## SPRAY-WELD ALLOYS

Arthur P. Shepard, Flushing, N.Y., assignor to Metalizing Engineering Co. Inc., a corporation of New Jersey

No Drawing. Application November 25, 1957  
Serial No. 698,378

16 Claims. (Cl. 75—5)

This invention relates to new and useful improvements in spray-weld alloys and in particular in nickel-base and cobalt-base alloys used in the spray-weld process. Such alloys are known in the art, and they contain boron or boron plus silicon to provide fluxing properties. For this reason these alloys are known as "self-fluxing alloys" and will be hereinafter referred to as such.

Such alloys are used for welding and brazing and particularly for coating materials applied as a fused or welded over-lay on base materials, such as steel or steel alloys.

The elements boron and silicon, when added to nickel or nickel base alloys, and cobalt or cobalt base alloys, act as fluxer of the alloy and of the surface to be alloyed during the fusing of the alloy when performing the brazing, welding or coating operation. Boron alone may be used in some cases, but superior fluxing action is usually obtained when both boron and silicon are used.

One process frequently used for applying fused coatings of self-fluxing alloys is known as "spray-welding." Spray-welding comprises the steps of first metal spraying the alloy onto the surface to be coated, and second, fusing the coating in place. The metal spraying operation can be carried out by any of the known metal spraying techniques, in which the material to be sprayed is fed into a heating zone where it is melted or heat-softened and from which it is, in finely divided form, propelled in molten or heat-plastic condition onto the surface to be coated. The material being fed to the heating zone may be in the form of a rod or in the form of a powder, or in some cases, in the form of a powder bonded together by a plastic material to form a wire, said plastic material being of a nature such that it disintegrates in the heat of the flame, releasing the metal particles. In metal spraying methods where the material is fed in the form of a rod or wire, the tip of the wire is melted in the heating zone and sufficient energy is applied to the tip of the molten wire by a blast of air or other gas, to cause the molten metal at the tip to subdivide into a fine spray.

After coatings have been applied by the metal spraying process, they are thereafter fused in the carrying out of the spray-welding process. Such fusing may be done in a furnace or, alternatively, by means of heating torches applied directly to the coated surface, or by other means such as induction heating.

The self-fluxing alloys heretofore most widely used in the spray-weld process comprise nickel or nickel-chromium alloys containing boron and silicon.

The extent to which the spray-welding properties of the boron, nickel-base alloy can remain essentially unaffected by the addition of certain alloy components is exemplified by the fact that they may contain from 0% up to 20% Cr by weight of total alloy. This component imparts increasing corrosion and oxidation-resistance properties without interfering with or displacing the essential properties of the alloy.

Elements such as carbon may be present in either nickel base or cobalt base alloys as impurities or as desir-

able components to increase, for instance, the hardness of the spray-welding alloy. The upper limit of carbon content, however, is dictated by the fact that excessive amounts will impart too high a degree of brittleness to the alloy, thereby interfering with the property of ductility. Another frequently occurring component of these spray-welding boron, nickel-base or cobalt base alloys is iron, which should not be normally present in amounts exceeding 10%, and preferably not in amounts exceeding 5% by weight of the total alloy.

A typical spray-weld alloy of the boron, nickel type, as an example, consists of 0.7—1% carbon, 3.5—4.5% silicon, 2.75—3.75% boron, 3—5% iron, and optionally an additional 16—18% chromium, with nickel making up the balance.

Some other spray-weld alloys of the boron, nickel type, which have been found suitable for the spray-weld process, are listed in the following table, the amounts indicating percent by weight:

TABLE

|                      |      |         |         |         |           |
|----------------------|------|---------|---------|---------|-----------|
| Si                   | 1-6  | 4-5     | 4-5     | 4-5     | 3.5-4.5   |
| B                    | 1-6  | 3.5-4.5 | 3.5-4.5 | 3.5-4.5 | 3.75-3.75 |
| Cu                   | 0-8  | 5-6     | 5-6     | 5-6     | 5-6       |
| Mo                   | 0-10 | 4.5-5.5 | 4.5-5.5 | 4.5-5.5 | 4.5-5.5   |
| Cr                   | 0-20 | 8-12    | 15-18   | 16-18   |           |
| C                    | 0-1  | 0-0.2   | 0-0.2   | 0-0.2   | 0-7-1     |
| Fe                   | 0-5  | 0-5     | 0-5     | 0-3     | 0-5       |
| Balance in all cases |      |         |         |         |           |
| Ni                   |      |         |         |         |           |

Cobalt base alloys can also be used as self-fluxing alloys for the spray-weld process in place of nickel base alloys. Some typical spray-weld alloys of the boron, 35 cobalt type, or of the boron-cobalt-nickel type, which have been found suitable for the spray-weld process, are listed in the following table:

TABLE

|    | Nominal Composition (% by weight) |         |         |         |         |
|----|-----------------------------------|---------|---------|---------|---------|
|    | Cr                                | Ni      | Co      | W       | C       |
| 45 | 0                                 | 0       | 30-35   | 16-20   | 16-20   |
|    | 0-30                              | 30-70   | 60-65   | 42-46   | 25-30   |
|    |                                   |         |         | 16-20   | 35-45   |
|    |                                   |         |         | 8-12    | 35-45   |
|    |                                   |         |         |         |         |
| 45 | 0-20                              | 4-5     | 0.3-1.5 | 2-2.5   | 0-0.4   |
|    |                                   |         |         |         | 0-0.4   |
|    |                                   |         |         |         |         |
|    |                                   |         |         |         |         |
| 50 | 0-4                               | 1.5-2.5 | 1.5-2.5 | 2.5-4.5 | 2.5-4.5 |
|    | 1.5-4                             | 0-8     |         | 2.5-3.5 | 2.5-3.5 |
|    |                                   |         |         | 4-8     | 4-8     |
|    |                                   |         |         |         |         |

Such heretofore known alloys have been subject to one serious defect, to more or less degree. This defect is that after fusing, small isolated pores appear occasionally in the coatings and are frequently uncovered by a finishing or grinding operation. Under certain circumstances these pores may have a random distribution and may appear fairly infrequently throughout the coating. Nevertheless, the appearance of even one pore uncovered by the grinding or finishing operation may be a very serious matter, and for many parts for which such coatings are used, such as pump plungers, may render the part totally defective and unusable. It is obvious therefore that even randomly distributed small pores can cause expensive loss of parts, particularly where large areas or a large number of parts are being spray-welded.

Under certain conditions pores in the finished coating may be distributed in systematic arrangements, as the result of the contour of the part being coated and the spraying technique used. In such cases clusters of pores appear at such locations as shaft shoulders or in lines over the grooves of V threads, where threading has been used as a means of undercutting and preparation of the

base for the application of the coating. In all such cases where clusters of pores appear near the surface, they are almost sure to render the finished part defective.

While it has been determined that spraying techniques, and base preparation techniques, can have an effect upon the number and location of pores produced, no combination of techniques has been discovered which will eliminate pores altogether.

One object of this invention is to provide a spray-welding powder of the self-fluxing type, which produces pore-free coatings when used in the normal operation of spray-welding.

It is a further object of the invention to provide such a spray-welding powder which will produce pore free spray-welded coatings, even though the coatings are sprayed under adverse conditions and without strict adherence to normal techniques, thereby providing a more trouble-free spray-welding process.

It is a further object of the invention to provide such a spray-welding powder for producing spray-welded coatings, which is not affected by a wide variety of relatively adverse base preparation techniques and still provide a pore-free alloy coating, thereby providing a more trouble-free spray-welding process.

It is a still further object of the invention to provide such a spray-welding powder suitable for producing pore-free spray-welded coatings and still retain all of the properties normally required of such alloys such as the following properties:

(1) The property of a melting point appreciably below the melting point of the base to which they are applied, which is usually steel;

(2) The property of wetting the surface to which they are applied, which is usually steel;

(3) The property of having a relatively wide viscous fluid range with respect to temperature variation so that the coatings will not run or drip during the fusing operation;

(4) The property of having a relatively low surface tension to avoid retraction from edges during the fusing operation;

(5) The property of having sufficient plasticity at temperatures below but near the melting point, to avoid undue cracking due to shrinkage during freezing;

(6) The property of having sufficient ductility or toughness to avoid cracking due to temperature variations during cooling;

(7) The property of forming an oxide-dissolving slag separable from the molten metal to remove the oxides therefrom, since such oxides formed during spraying or fusing interfere seriously with the coalescence during fusing and adversely affect the physical properties of the fused coatings;

(8) The property of resisting corrosive attack of various environments.

These and still further objects will become apparent from the following description.

Spray-welding powder for use in the spray-welding process in accordance with this invention comprises any conventional spray-welding powder of the self-fluxing type additionally containing a minor quantity of at least 0.2% aluminum. Such aluminum may be either an alloy constituent of the self-fluxing type alloy or added to the powder in other form, such as in the form of aluminum powder. Alternatively, the aluminum may be added in the form of an alloy or combination with another element or elements, such as, for instance, ferro aluminum; provided that such other element or elements do not adversely affect the performance of the powder mixture in the spray-welding process.

It is preferred to add the aluminum to a boron, nickel-base, cobalt-base, or nickel/cobalt-base alloy in the form of an alloying element with a percentage of from 0.2 to 0.4% by weight.

It is sometimes preferred to mix two or more alloys

in powder form to produce a powder mixture in which one or more of the constituents contain sufficient boron or boron and silicon to perform the self-fluxing function for the entire mixture when the mixture is spray-welded.

5 In such cases it is preferred to add the aluminum to one or more of the alloy constituents, such that the percentage of aluminum in the total mixture of powder is between 0.2 and 2%. Alternatively, the aluminum may be added to such a mixture in the form of a powder or alloyed in another alloy with element or elements which are compatible with such mixture.

It has been found that at least substantially 0.2% of aluminum is required as an addition by weight of the total self-fluxing alloy powder, in accordance with this invention, to perform the necessary function of eliminating pores from the ultimately fused spray-welded coating.

There is no upper limit at which the aluminum ceases to perform its function of eliminating the pores from the fused spray-welded coating formed. In general, however,

20 only a minor quantity of aluminum should be used since in most cases it is desirable for the aluminum to merely serve the function of eliminating the pores without affecting the powder in any other manner. Amounts of aluminum in excess of about 5% by weight of the powder generally adversely affect the fusing characteristics of the powder. When amounts of aluminum of more

25 than about 2% by weight of the total powder are used, the same affects the appearance of the fused coating ultimately formed, giving the same a dull and tarnished looking surface. Therefore, for many applications it is desirable to use less than 2% by weight of the aluminum. The preferable range of amount of aluminum is between 0.2-0.4% by weight, since when used in this amount the aluminum effectively eliminates the pores without affecting the properties of the powder in any other manner.

30 In general, however, larger amounts of aluminum may be added without affecting the other characteristics of the powder when the aluminum is added as an alloying element to the self-fluxing type alloy than when the aluminum is added as aluminum powder in admixture with the remainder of the spray-weld powder.

In cases where the aluminum is alloyed it is often possible to safely use amounts of 0.2-1% without any danger of affecting the normal properties of the powder and without the danger of causing a dulling of the finished surface from the spraying and fusing of the coating.

35 The spray-weld powder should in general have a mesh size below 100 U.S. standard. The exact mesh size generally depends on the particular equipment used for the spraying and the particular fuel gas. Thus, for example, when using acetylene as the fuel gas, the particles should all be below about 120 U.S. standard mesh and not more than 15% of the particles should be below 50 325 mesh. In contrast to this, when using hydrogen as a fuel gas, there is no lower limit as to the mesh size and all the particles may be below 325 mesh, i.e. may be as small as it is physically possible to obtain.

40 The use of aluminum as a de-oxidant, as an alternative to other well known de-oxidizing materials, by adding it to the melt in the manufacture of alloys of the boron, nickel-base or cobalt-base types has been well known in the art. As the result of this practice, small traces of aluminum have sometimes appeared in spray-weld alloys of the type used for spray-welding, and in some cases residual amounts of aluminum resulting from this manufacturing practice have been found in percentages up to substantially 0.1%. In no cases, however, have the residual traces of aluminum, even including those cases where the residual aluminum has been found in an amount of substantially 0.1%, formed a mixture or alloy which produced pore-free spray-welded coatings.

45 The following are some examples of alloy powders

and alloy powder mixtures in accordance with this invention:

*Example 1*

An example of a spray-weld alloy powder in accordance with this invention is a powder substantially all minus 120 mesh U.S. standard screen size and containing not more than 20% minus 325 U.S. standard screen size, the particles of the powder being of a boron, nickel type alloy consisting of 0.7-1% carbon, 3.5-4.5% silicon, 2.75-3.75% boron, 3-5% iron, and optionally an additional 16-18% chromium, 0.2-2% aluminum with nickel making up the balance.

*Example 2*

Another example of a spray-weld alloy powder in accordance with this invention is a powder substantially all minus 120 mesh U.S. standard screen size and containing not more than 20% minus 325 U.S. standard screen size, the particles of the powder being of a boron-cobalt type alloy consisting of 0.5-1.5% carbon, 1.5-2.5% boron, 4-5% iron, and optionally an additional 26-30% chromium, 0.2-2% aluminum with cobalt making up the balance.

*Example 3*

Still another example of a spray-weld alloy powder in accordance with this invention is a powder substantially all minus 120 U.S. standard screen size and containing not more than 20% minus 325 U.S. standard screen size, the powder consisting of a 50%-50% mechanical mixture of metal particles of a first and second alloy, the first alloy consisting of 0.7-1% carbon, 3.5-4.5% silicon, 2.75-3.75% boron, 3-5% iron, and optionally an additional 16-18% chromium with nickel making up the balance; the second such alloy consisting of 1-6% silicon, 1-6% boron, 3-8% copper, 3-10% molybdenum, 0.4-4% aluminum and optionally an additional 16-20% chromium, 0-1% carbon, 0-5% iron with nickel making up the balance. It should be noted that in this particular mixture of powder alloys, the percentage of the aluminum appearing in the mixture in accordance with the invention is 0.2-2%, due to the fact that it occurs in one 50% constituent in the range 0.4-4%.

*Example 4*

Still another example of a spray-weld alloy powder in accordance with this invention is a powder substantially all minus 120 mesh U.S. standard screen size and containing not more than 20% minus 325 U.S. standard screen size, the particles of the powder being a mixture of powder particles of a boron, nickel type alloy, consisting of 4-5% silicon, 3.5-4.5% boron, 5-6% copper, 4.5-5.5% molybdenum, 8-12% chromium, 0-0.2% carbon, 0-5% iron with nickel making up the balance; and a pure powder aluminum in sufficient quantity to provide 0.2-2% by weight of the entire mixture.

The following example illustrates the use of a spray-weld powder in accordance with this invention:

*Example 5*

One alloy in accordance with this invention has the following analysis:

| Element:   | Percent |
|------------|---------|
| Carbon     | 0.1     |
| Silicon    | 4.5     |
| Boron      | 3.75    |
| Molybdenum | 5       |
| Iron       | 2       |
| Copper     | 5.5     |
| Chromium   | 15.5    |
| Aluminum   | 0.3     |
| Nickel     | Balance |

In one method of applying the alloy exemplified by the above specified analysis, it is subdivided so that it

will all pass through a 120 mesh standard screen and applied by means of conventional-powder-metal spray gun. As a specific example of this application, a steel shaft having a 2" diameter section 4" long, and with a keyway  $\frac{1}{8}$ " x  $\frac{1}{4}$ " x 1" long at one end of the section to be sprayed, is prepared for the spray-welding operation by first machining the surface to be coated with a V-thread approximately 30 threads to the inch and with a depth of approximately 75% of full U.S. standard depth and thereafter grit-blasting with a conventional blast machine, in which the grit is blown forcibly against the surface of the shaft by means of compressed air, using S.A.E.G. -16 crushed steel grit and a blast air pressure of 100 p.s.i. for a few minutes, sufficiently to roughen and thoroughly clean the surface to be coated. A steel key,  $\frac{1}{4}$ " square, is fitted into the keyway of the shaft before blasting.

A coating of  $\frac{1}{6}$ " thickness of the alloy is metal-sprayed in conventional manner over the entire shaft section to be coated while the shaft is rotated in a lathe. The key is then removed by grinding away the edges of the sprayed coating adjacent the key and tapping the key out of the keyway.

While rotating the shaft in a lathe, the shaft is preheated, using a conventional oxy-acetylene heating torch over the entire coated section, to a temperature of approximately 1000° F. The torch is then concentrated at one end of the coated section while the shaft is still rotating, so as to raise the temperature of a small band of the coating. As the coating fuses, the torch is gradually moved along the coated section of the shaft so as to successively fuse each small band of the coating until the entire coating has been fused. The heating is then stopped and the shaft allowed to cool in air and without any attempt at controlled cooling or heat-insulation.

The coated end of the shaft is then ground to a diameter of approximately  $2\frac{3}{16}$ ". The coating will shrink about 20% during fusing from the original sprayed thickness of  $\frac{1}{6}$ ". This will still leave sufficient finish allowance for grinding the coating to a finished thickness of approximately  $\frac{3}{32}$ " on a side of the shaft.

The coating thus applied was found to be completely finish-ground on the diameter, have a relatively small radius on the corner at the edge of the keyway, be firmly adherent at the edges of the keyway, as well as elsewhere, and be free from pores in its entire surface.

The spray-weld powder in accordance with this invention is for use in a metal spray gun and may ordinarily be used in a powder type metal spray gun directly without further treatment. However, if it is desired to use the powder in accordance with the invention in a wire type metal spray gun, this may be done, in accordance with known practice as previously described, by binding the particles of powder together with a suitable plastic binder in the form of a rod or wire. The term "powder" is used in the claims to generally designate the powder both in loose form and in bound form as for example in the form of a rod or wire.

*Example 6*

Example 5 was repeated except prior to use, the powder was intimately mixed and dispersed in a melt of high pressure polyethylene so that the melt contained 15% by weight of polyethylene and 85% by weight of the powder. The melt was then extruded into the form of a wire and the spraying was effected with a conventional wire type metal spray gun. In all other respects, conditions and results obtained were identical to Example 5.

The foregoing specific description is for purposes of illustration and not of limitation and it is therefore my intention that the invention be limited only by the appended claims or their equivalents wherein I have endeavored to claim broadly all inherent novelty.

I claim:

1. In a spray-weldable, self-fluxing metal powder essentially consisting of a base metal selected from the group consisting of nickel, cobalt and combinations thereof, and containing boron as the self-fluxing element, the improvement which comprises the powder additionally containing about 0.2-5% by weight of aluminum.
2. Improvement according to claim 1 in which said aluminum is alloyed with at least one other constituent of said powder.
3. Improvement according to claim 1 in which said aluminum is present in unalloyed, divided form.
4. Improvement according to claim 1 in which the metal powder has a particle size below about 100 mesh.
5. In a spray-weldable, self-fluxing nickel base alloy metal powder containing boron as the self-fluxing element, the improvement which comprises the alloyed metal powder additionally containing about 0.2-5% by weight of aluminum.
6. Improvement according to claim 5 in which said aluminum is present in amount of about 0.2-2% by weight.
7. Improvement according to claim 5 in which said aluminum is alloyed with at least one of the other constituents of said powder.
8. Improvement according to claim 5 in which said aluminum is present in an unalloyed, divided form.
9. Improvement according to claim 5 in which said powder has a particle size below about 100 mesh.
10. In a spray-weldable, self-fluxing nickel-cobalt base alloy metal powder containing boron as the self-fluxing element, the improvement which comprises the alloy metal powder additionally containing about 0.2-5% by weight of aluminum.
11. In a spray-weldable, self-fluxing cobalt base alloy metal powder containing boron as the self-fluxing element, the improvement which comprises the alloy metal

powder additionally containing about 0.2-5% by weight of aluminum.

5 12. Improvement according to claim 11 in which said aluminum is present in amount of about 0.2-2% by weight.

13. Improvement according to claim 11 in which said aluminum is present in unalloyed, divided form.

14. Improvement according to claim 11 in which said powder has a particle size below about 100 mesh.

10 15. A spray-weldable alloy powder of the nickel base type comprising 0.7-1% carbon, 3.5-4.5% silicon, 2.75-3.75% boron, 3-5% iron, up to 18% chromium, 0.2-2% aluminum and nickel making up the balance.

15 16. A spray-weldable alloy powder of the cobalt base type comprising 0.5-1.5% carbon, 1.5-2.5% boron, 4-5% iron, up to 30% chromium, 0.2-2% aluminum and cobalt making up the balance.

References Cited in the file of this patent

UNITED STATES PATENTS

|           |                   |               |
|-----------|-------------------|---------------|
| 1,365,499 | Kelley            | Jan. 11, 1921 |
| 1,514,064 | Mandell           | Nov. 4, 1924  |
| 2,103,267 | Mandell           | Dec. 28, 1937 |
| 2,504,239 | Rochl             | Apr. 18, 1950 |
| 2,661,285 | Gorschalki        | Dec. 1, 1953  |
| 2,714,760 | Boam et al.       | Aug. 9, 1955  |
| 2,743,177 | Cape              | Apr. 24, 1956 |
| 2,775,531 | Montgomery et al. | Dec. 25, 1956 |
| 2,793,108 | Franklin          | May 21, 1957  |
| 2,864,696 | Foreman           | Dec. 16, 1958 |
| 2,868,667 | Bowles            | Jan. 13, 1959 |
| 2,875,043 | Tour              | Feb. 24, 1959 |

OTHER REFERENCES

35 Holgate: Electroplating and Metal Spraying, vol. 7, No. 6, June 1954, pages 239-242 and 245. Published by Robert Draper, Ltd., Teddington, Middx., England.